

# UNITED STATES PATENT OFFICE.

JEAN V. SKOGLUND, OF NEW YORK, N. Y.

## FIRE AND WATER PROOF COMPOSITION AND PROCESS OF MAKING SAME.

1,194,558.

Specification of Letters Patent. Patented Aug. 15, 1916.

No Drawing.

Application filed August 15, 1913. Serial No. 784,898.

To all whom it may concern:

Be it known that I, JEAN V. SKOGLUND, a citizen of the United States, and a resident of the borough of Brooklyn, county of Kings, city and State of New York, have invented a certain new and useful Fire and Water Proof Composition and Process of Making Same, of which the following is a description in such full, clear, and exact 10 terms as will enable any person skilled in the art to which it pertains to make and use the same.

My invention relates to the manufacture of a fire and waterproof composition suitable, for example, for application to such woods as balsa wood which are soft and spongy and unfit to be covered with ordinary paint, which composition shall be both fire and waterproof and at the same time 15 with sufficient body and stiffness or strength to resist the crushing and chipping strains to which the coated wood will be subjected when in use, for example, as life preservers, life rafts and the like. For coating such 20 woods to prevent them from absorbing moisture, I have found that the covering or coat cannot be ordinary paint for the wood will absorb too much of the paint and become too heavy and dense for use as a buoy- 25 ant body or for heat-insulation and the paint is not sufficiently hard to resist the crushing strains on the soft, spongy wood. The covering, therefore, must be of such material as will offer a firm resistance and protect the soft wood not only from absorption, 30 but from crushing or denting. Hydrocarbons such as pitch, tar, asphalt and other similar materials are suitable for this purpose but are so inflammable that they can- 35 not ordinarily be used. My invention deprives these materials of their inflammable character.

The invention, of course, has other uses than those above outlined and is in no sense 40 limited to the same, but may be employed in any situation where a fire and waterproof coating is required for either wood or metal. In carrying out my invention I treat tar, pitch or similar materials with bromin, 45 which combines with them and forms a brominated product. This compound is non-inflammable and when subjected to heat melts and forms a protective coating for the material on which it is applied.

Instead of using tar, pitch, etc., I may 50 combine the bromin with a refined and dis-

tillated product of the same. Such products are well known, but creosote-oil, anthracene and naphthalene may be mentioned. Sometimes it will be more convenient to apply the 55 bromin first to a fluid product such as tar, dead oil, etc., and then combine the mixture with a solid material such as pitch, asphaltum, etc., though the bromin may be mixed directly with the tar or pitch if desired. 60

One method of carrying out my invention is to take about two (2) parts of bromin and mix the same with four (4) parts of gas tar or dead oil. This sets up a very active reaction accompanied by heat and ebullition 65 and from which some acid vapor is given off. The reaction finally subsides and the resultant compound is then mixed and fused with about twenty (20) parts of pitch. 70

The compound should be heated to about 75 the fusing point and applied when heated to the surface to be covered. Accordingly in this practice the compound is subjected to repeated heatings and coolings which act on the same to raise its fusing point and in 80 order to avoid high temperatures I may treat the compound from time to time with further additions of bromin and dead oil. That is to say, after a certain quantity of the composition has been formed in either of 85 the ways above mentioned and heated up for use from time to time, that which remains, upon requiring increased heat to fuse it, may have a mixture of bromin and dead oil added to soften it or reduce its fusing 90 point and in this manner the fusing point kept down within easy working limits.

The bromin does not destroy the waterproofing and protective qualities of the tar, pitch or other similar materials, but it does 95 modify them so that they may be ignited and will burn with such difficulty only that they may be regarded as practically fireproof. The composition makes a tough, 100 elastic protective coat for all materials which usually require to be coated and it is, as explained, both waterproof or non-absorbent and fireproof. I may also mix a brominated substance as above described with any kind of oil and pigments to form 105 a paint which may be used for any purpose when it is desirable to make it fireproof.

Having thus described my invention, what I claim as new and desire to secure by Letters Patent of the United States is:—

1. A fire-and waterproof composition for use as a covering or coating material con-

65

70

75

80

85

90

95

100

105

110

taining a heavy hydrocarbon and dead oil combined with bromin substantially as and for the purpose specified.

2. The process of making a fire-and water-proof composition which consists in combining dead oil and bromin and then combining the same with a heavy hydrocarbon substantially as and for the purpose specified.

In testimony whereof I have hereunto signed my name in the presence of two witnesses. 10

JEAN V. SKOGLUND.

Witnesses:

SYDNEY H. GIELLERUP,  
ARTHUR VEHLOW.